

## UNITED STATES PATENT OFFICE

2,084,950

## COMPRESSION OF FLUORINATED HYDRO-CARBONS

Frederick Baxter Downing, Carneys Point, and Anthony Francis Benning, Pennsgrove, N. J., assignors to E. I. du Pont de Nemours & Company, Wilmington, Del., a corporation of Delaware

No Drawing. Application March 26, 1935,  
Serial No. 13,174

11 Claims. (Cl. 62—178)

This invention relates to gas compression, more particularly to the compression of gaseous fluorinated hydrocarbons, and to a method of lubrication during such compression.

5 Gaseous fluorinated aliphatic hydrocarbons, particularly the fluorochloro hydrocarbons, have recently found rather wide use as refrigerants. These compounds, while advantageous in many respects, have a definite disadvantage over the 10 strongly polar refrigerants such as sulfur dioxide and ammonia in that they are generally miscible in all proportions with hydrocarbon lubricating oils. This property is disadvantageous because in a refrigeration system where the reserve supply of lubricant is in contact with the refrigerant vapor, the oil will dissolve the refrigerant resulting, particularly during shutdowns, in all of the refrigerant collecting in the oil reserve chamber. When now the machine is started up, violent ebullition of the refrigerant 15 from the oil carries the lubricant with it into other parts of the system, leaving the compressor without sufficient oil to operate properly. This, of course, causes undue wear. Hence, under 20 such conditions of operation, some means must be provided for the return of the lubricant to the compressor. In the case of sulfur dioxide and ammonia, the oil dissolves but a small quantity of refrigerant and the difficulty described 25 above is not encountered.

It is an object of the present invention to provide a method of compressing gaseous fluorinated aliphatic hydrocarbons under new and improved lubricating conditions. A further object is to provide a method of compressing gaseous fluorinated aliphatic hydrocarbon refrigerants in the ordinary type of refrigeration system wherein the reserve supply of lubricant is in contact with the refrigerant vapor, characterized 30 by the use of a lubricating fluid which has good lubricating properties and which does not tend to dissolve excessive amounts of the fluorinated aliphatic hydrocarbon. More specific objects are 35 to accomplish the foregoing objects with fluorochloro aliphatic hydrocarbons, and more particularly difluorodichloromethane. Other objects will appear hereinafter.

These objects are accomplished by employing 40 liquid organic esters of phosphorus acids as lubricants in systems for the compression of fluorinated aliphatic hydrocarbons.

The invention will be further illustrated but 45 is not limited by the following examples.

## Example I

Difluorodichloromethane was compressed in the type of compressor ordinarily employed in household refrigerators using technical tricresyl phosphate as a lubricant. The proportions of technical tricresyl phosphate corresponded with the volume proportions of oil normally employed in the usual sulfur dioxide household refrigerator compressor. Excellent results were obtained. The difluorodichloromethane was not miscible 5 with the technical tricresyl phosphate as in the case of oil, and although a study of the solubility properties of tricresyl phosphate, as given below, indicates that some of the fluorochloro hydrocarbon will be dissolved by the organic phosphate ester, nevertheless this solvent action did not interfere with the operation of the compressor and highly satisfactory results were obtained both before and after shut-downs. No undue wear on the compressor parts was evident.

20 Good results were also obtained in the compression of difluorodichloromethane in a large-size compressor.

Technical tricresyl phosphate is a mixture of the esters and mixed esters of the isomeric cresols. 25 Methods of obtaining it are known in the art. One method, for example, is to react a technical mixture of the isomeric cresols with phosphorous oxychloride.

30 Some of the properties of this material which affect its use for the purpose described above are given below:

## Properties of technical tricresyl phosphate pertinent to its use as a lubricant for fluorinated hydrocarbons

|                                                                |        |
|----------------------------------------------------------------|--------|
| Saybolt viscosity at 100° F.—seconds                           | 120    |
| Saybolt viscosity at 210° F.—do—                               | 39.6   |
| Viscosity index                                                | 50     |
| Pour point—degrees F.                                          | —20 40 |
| Pour point saturated with $CF_2Cl_2$ —do—                      | —20    |
| Flash point (open cup)—do—                                     | 475    |
| Fire point—do—                                                 | 620    |
| Almen film strength—lbs. per sq. in                            | 30,000 |
| Solubility in $CF_2Cl_2$ (77° F.)—per cent                     | 12 45  |
| Solubility $CF_2Cl_2$ in tricresyl phosphate (77° F.)—per cent | 45     |

Of the properties given above, the high Almen film strength and non-miscibility with fluorochloro hydrocarbons may be noted as being especially desirable.

## Example II

Instead of difluorodichloromethane, mono-

fluorotrichloromethane may be compressed as in Example I with correspondingly good results.

*Example III*

5 Tetrafluorodichloroethane may be compressed as in Example I with good results.

Similarly, the invention may be applied to the treatment of other gaseous fluorinated aliphatic hydrocarbons, as described, for example, in 10 Midgley, Henne and McNary, Reissue Patent No. 19,265, dated August 7, 1934.

Instead of technical tricresyl phosphate, other liquid organic esters of phosphorus may be employed as, for example, any of the following: tri- 15 (ortho-cresyl) phosphate; tri-(meta-cresyl) phosphate; tri-(para-cresyl) phosphate; phenyl-di-(ortho-, meta-, or para-cresyl) phosphates; mixed isomeric di-cresyl-phenyl phosphates; di- 20 (ortho-, meta-, or para-cresyl)-xylene phosphates and mixed isomeric phosphates; trixylenol phosphates; octyl-lauryl phosphate; dioleyl phosphate; dioctyl phosphate; mono- and dilorol phosphates; mono- and diocenol phosphates; phosphate esters of oenol; mixed tertiary amyl- 25 phenyl phosphates; lorol-cresyl phosphate; and liquid mixtures of any of the foregoing phosphorus esters with any of the following: dilauryl phosphate, dicetyl phosphate, distearyl phosphate, dimyristyl phosphate, dibutyl phosphate and dicyclohexyl phosphate. Similar liquid organic esters of phosphorus, thiophosphoric, meta-phosphoric and pyrophosphoric acids and mixtures containing them may be used. In general, we prefer to employ the neutral and acidic 30 esters of the phosphorus acids.

The term "lorol" is used to describe a mixture of esters or mixed esters derived from a mixture of alcohols containing mostly lauryl alcohol but also containing some decyl and myristyl alcohols. 40 The term "oenol" is applied to a mixture of primary aliphatic alcohols having 12 to 18 carbon atoms and consisting mainly of oleyl alcohol. Such a mixture usually has an iodine value of about 50.

45 A preferred class of the organic phosphorus esters may be represented by the following general formula:



where X, Y and Z represent —H or lower aliphatic hydrocarbon radicals such as methyl, ethyl, isopropyl and butyl but may not all be —H at the same time, and m, n, and o are 1, 2 or 3.

65 Another preferred class of organic phosphorus esters for our purpose are the normally liquid long chain aliphatic hydrocarbon mono- and diesters of phosphorus acids preferably having at least one carbon chain of eight or more carbon atoms, e. g., dioctyl phosphate, mono- and dilorol phosphates, mono- and diocenol phosphates, and octyl-lauryl phosphate.

70 A third preferred class of compounds are the normally liquid mixed aliphatic-aromatic di-

esters of phosphorus acids, as, for example, mixed tertiary amyl-phenyl phosphate and lorol-cresyl phosphate.

75 The liquid organic esters of phosphorus acids are preferably employed in undiluted state, that is, without the addition of material amounts of solvents or diluents, particularly those diluents which are poorer lubricants or tend to dissolve the fluorinated aliphatic hydrocarbon. If any dilution is to be made non-polar lubricants rather than polar lubricants are preferred. Thus, polar lubricants typified by polyhydric alcohols such as glycerin are not as good lubricants as the organic phosphorus esters typified by tricresyl phosphate.

10 This invention has been instrumental in solving one of the more difficult problems in the compression of fluorinated hydrocarbons, particularly in the field of household refrigeration. It has also been satisfactorily used in larger scale compression systems.

15 As many apparently widely different embodiments of this invention may be made without departing from the spirit and scope thereof, it is to be understood that we do not limit ourselves to the specific embodiments thereof except as defined in the appended claims.

20 We claim:

1. The method of compressing gaseous fluorinated aliphatic hydrocarbons which comprises compressing the gaseous fluorinated hydrocarbons in the presence of lubricants consisting of liquid organic esters of phosphorus acids, said liquid organic esters being substantially immiscible with the fluorinated aliphatic hydrocarbons.

30 2. The method of compressing gaseous difluorodichloromethane which comprises compressing the difluorodichloromethane in the presence of a lubricant consisting of liquid organic esters of phosphorus acids having the following general formula.



where X, Y and Z represent —H or lower aliphatic hydrocarbon radicals but may not all be —H at the same time, and m, n, and o are 1, 2 or 3.

55 3. The method of compressing gaseous difluorodichloromethane which comprises compressing the difluorodichloromethane in the presence of a lubricant consisting of technical tricresyl phosphate.

60 4. The method of compressing gaseous fluorinated hydrocarbons which comprises compressing the gaseous fluorinated hydrocarbons in the presence of normally liquid long chain aliphatic hydrocarbon mono- and di-esters of phosphorus acids.

65 5. The method of compressing gaseous fluorinated hydrocarbons which comprises compressing the gaseous fluorinated hydrocarbons in the presence of normally liquid mixed aliphatic-aromatic di-esters of phosphorus acids.

70 6. The process of compressing gaseous fluorinated hydrocarbons which comprises compress-

5

10

15

20

25

30

35

40

45

50

55

60

65

70

75

ing the gaseous fluorinated hydrocarbons in the presence of liquid organic esters selected from the class consisting of aromatic di- and tri-esters of phosphorus acids, normally liquid long chain aliphatic hydrocarbon mono- and di-esters of phosphorus acids, and normally liquid mixed aliphatic-aromatic esters of phosphorus acids.

7. In the process of refrigeration which comprises condensing a gaseous fluorinated hydrocarbon refrigerant and then evaporating the same, the step which comprises compressing said refrigerant in the presence of liquid organic esters of phosphorus acids which are substantially immiscible in said refrigerant.

8. In the process of refrigeration which comprises condensing a gaseous fluorinated hydrocarbon refrigerant and then evaporating the same in the vicinity of a body to be cooled, the step which comprises compressing said refrigerant in the presence of liquid organic esters selected from the class consisting of aromatic di- and tri-esters of phosphorus acids, normally liquid long chain aliphatic hydrocarbon mono- and di-esters of phosphorus acids, and normally liquid mixed aliphatic-aromatic esters of phosphorus acids.

9. In the process of refrigeration which comprises condensing a gaseous fluorinated hydrocarbon refrigerant and then evaporating the same, the step which comprises compressing said refrigerant in the presence of a lubricant con-

sisting of liquid organic esters of phosphorus acids having the following general formula



where X, Y and Z represent —H or lower aliphatic hydrocarbon radicals but may not all be —H at the same time, and m, n and o are 1, 2 or 3.

10. In the process of refrigeration which comprises condensing a gaseous fluorinated hydrocarbon refrigerant and then evaporating the same, the step which comprises compressing said refrigerant in the presence of a lubricant consisting of technical tricresyl phosphate.

11. The process of refrigeration which comprises compressing a gaseous fluorinated hydrocarbon refrigerant in the presence of a lubricant consisting of liquid organic esters of phosphorus acids which are substantially immiscible in said refrigerant, condensing said refrigerant, and then evaporating the same in the vicinity of a body to be cooled.

FREDERICK BAXTER DOWNING.  
ANTHONY F. BENNING.